

# UNITED STATES PATENT OFFICE.

CHARLES MILTON STINE, OF CHESTER, PENNSYLVANIA, ASSIGNEE, BY MESME ASSIGNMENTS, TO E. I. DU PONT DE NEMOURS AND COMPANY, A CORPORATION OF DELAWARE.

## COMPOSITION FOR DETONATORS.

1,313,650.

Specification of Letters Patent. Patented Aug. 19, 1919.

No Drawing.

Application filed December 18, 1918. Serial No. 806,416.

To all whom it may concern:

Be it known that I, CHARLES MILTON STINE, of Chester, in the county of Delaware, and in the State of Pennsylvania, have invented a certain new and useful Improvement in Compositions for Detonators, and do hereby declare that the following is a full, clear, and exact description thereof.

The object of my invention has been to provide an improved composition for detonators and which shall have among others the advantages of having a high velocity of detonation and of being capable of detonating violently and with a sufficient power to cause the detonation of explosives not easily detonated.

To such ends my invention consists in the detonator composition, that is to say different types of blasting caps hereinafter specified. I have discovered that certain hemi or pseudo celluloses such as the seeds of certain tropical palms known as "vegetable ivory," when suitably treated, have a high velocity of detonation which especially fits them for use as initial igniters of many types and particularly for use in caps and detonating compositions, the caps being for instance blasting caps such as are used for the detonation of dynamite charges.

I have discovered for example that nitrated ivory nut mixed with such primary detonating compounds as mercury fulminate or lead azid and then pressed with an inverted capsule into shells which are used for blasting caps forms a powerful detonating composition, and that when the composition is ignited, as by means of a safety fuse, it detonates violently and with sufficient power to cause the detonation of dynamite. A suitable mixture is 90 parts of fulminate of mercury and 10 parts of nitrated ivory nut, or a mixture of 90 parts of lead azid and 10 parts nitrated ivory nut is equally powerful.

Not only is such nitrated ivory nut useful in the primary detonating composition, but I have discovered that the nitrated ivory nut, either alone or mixed with an oxidizing agent such as potassium chlorate, may be used as the main charge of the blasting cap or electric blasting cap, with a primary detonating composition such as those above described, or fulminate of mercury or lead azid without the nitrated ivory nut, or other

primary detonating composition. As an example, of such a main charge of a blasting cap, fifteen grains of nitrated ivory nut may be loaded in the usual manner into a copper shell such as is used for blasting caps and pressed in place by means of high pressure; six grains of a 90-10 mixture of fulminate of mercury and potassium chlorate may then be placed on top of the nitrated ivory nut and pressed into place at high pressure; the charge may then be covered with a perforated thimble or inverted capsule if desired. The blasting caps so formed may be ignited by the flame from a safety fuse in the usual way and will detonate with great violence.

Nitrated ivory nut may also be used in blasting caps in combination with organic nitro-compounds, either mixed with the nitro-compound or pressed into the cap shell in a separate charge. As an example of the use of nitrated ivory nut mixed with an organic nitro-compound, 10 grains of a mixture of equal parts of trinitrotoluene and nitrated ivory nut may be loaded in the usual manner into a copper shell and packed at high pressure. Seven (7) grains of fulminate of mercury are then placed on top of the pressed charge and also pressed into place at high pressure, with a perforated capsule placed on top of the primer. As an example of the use of nitrated ivory nut in combination with an organic nitro-compound, but not directly mixed with it, a cap may be loaded with 10 grains of trinitrotoluene or picric acid and primed with a mixture of 90 parts lead azid and 10 parts nitrated ivory nut, the main charge and primer being pressed either at the same time or separately.

While I have given specific examples of the use of nitrated ivory nut in detonator compositions, it is to be understood that my invention is not limited to any particular detonator composition nor to any specific methods of use in blasting or other caps, but that I desire to claim in the broadest manner the use of nitrated vegetable ivory and similar hemi and pseudo celluloses in detonator compositions.

I claim:

1. A detonator charge containing nitrated hemi-cellulose and a primer containing a primary detonating compound.

2. A detonator charge containing nitrated ivory nut and a primer containing a primary detonating compound.
3. A blasting cap charge containing nitrated hemi-cellulose and a primer containing a primary detonating compound.
4. A blasting cap charge containing nitrated ivory nut and a primer containing a primary detonating compound.
5. A detonating charge comprising a main charge of nitrated ivory nut, and primer containing a primary detonating compound and potassium chlorate.
6. A blasting cap charge comprising a main charge containing nitrated ivory nut and primer containing mercury fulminate.
7. A blasting cap charge comprising a main charge containing nitrated ivory nut, and a primer containing mercury fulminate and potassium chlorate.
8. A blasting cap charge comprising a main charge containing 15 parts of nitrated ivory nut and a primer containing 6 parts of a 90%—10% mixture of fulminate of mercury and potassium chlorate.

20 In testimony that I claim the foregoing I have hereunto set my hand.

25 CHARLES MILTON STINE.

Witnesses:

HENRY W. JONES,  
CLIFFORD E. BLYTHE.